

## UNITED STATES PATENT OFFICE.

ANTON WEINDEL, OF ESSEN-RUHR, GERMANY, ASSIGNOR TO ZECHE MATHIAS STINNES, OF ESSEN-RUHR, GERMANY.

## PROCESS OF OBTAINING LUBRICATING OILS AND PHENOLS FROM COAL TAR.

No Drawing. Application filed December 12, 1924, Serial No. 755,556, and in Germany December 27, 1923.

The primary tar or so-called "low temperature" tar obtained by distilling pit coal at low temperatures cannot be distilled without being decomposed. Even with the use 5 of a vacuum or steam or of both together, it is not possible to recover the materials present in the primary tar in an unaltered condition. This fact is of considerable importance because the viscous oils of the primary 10 tar which to a very great extent lose their viscous properties in consequence of the high temperatures of distillation.

I have succeeded in discovering methods by means of which primary tar is separated 15 into its components and the latter are recovered without their properties becoming altered. In the first instance the so called asphalt materials are separated from the crude primary tar by thoroughly mixing it 20 with the double to fourfold quantity of benzine and then agitating the mixture at the ordinary atmospheric temperature. By allowing the mixture to stand at the ordinary temperature or at a temperature reduced by 25 cooling, the asphalt after a short length of time is deposited in the shape of an insoluble mass whereupon the benzine-solution is poured off and the benzine completely removed by driving it off. The liquid oils which remain as a result of distillation 30 contain neutral oils free from asphalt and also contain the phenols of the primary tar. The separating of these two, the neutral oils from the phenols, is then effected by mixing them with a sufficient quantity of spirit (i. e., alcohol) of not over 60% strength and 35 by heating the mixture to a temperature of 70-75° C. After the mixture has been allowed to stand for a short time the phenols are dissolved by the dilute alcohol while the neutral oils remain undissolved. The two are then separately drawn off. The alcohol and a part of the water are then driven off 40 from the phenols by heating the aqueous and alcoholic solution to a temperature of about 95° C. whereby the previously dissolved phenols are precipitated. The neutral oils are also freed by heating from the slight quantities of alcohol which they have 45 taken up. Both products, the phenols and the neutral oils, are absolutely pure and ready for use. The phenols are preferably distilled again, especially if they are intended to be used for medicinal purposes. 50

The separation of the phenols by washing 55 the heated mixture with diluted alcohol is only effected in order to produce neutral oils free from phenol when such are required.

The neutral oils which are produced according to the process described in the foregoing have approximately the viscosity of 60 watch-maker's-oil. If with the object of increasing the viscosity one distills off a small percentage of the hydrocarbons of a 65 low boiling point for instance up to a boiling point of 220-250° C. at 760 mm, oils having the viscosity of a good fatty tar oil will be obtained. By this means however the solidifying point which previously was at -8 to 70 -10° C. is considerably increased (to about 0° C.). Naturally this circumstance affects the oils when oils of very low cold test are wanted.

In order to avoid this difficulty, I add to the primary tar free from asphalt after the 75 benzine has been driven off, approximately double the quantity of acetone and I cool the solution and stir it well whereby yellowish and slimy masses precipitate as being non-soluble in acetone or only very 80 slightly therein. The slimy material may be separated by filtration. The solution of the primary tar in acetone is then diluted with water at the ordinary temperature or preferably at slightly above ordinary temperature. In this manner the primary tar is completely divided into the 85 neutral oils which separate out and phenols soluble in the acetone solution. From the neutral oils only the acetone and a small 90 amount of water need to be driven off and they may be used directly as lubricating oils of a good solidifying point (-6 to -8° C.) The diluted solution of the phenol in acetone is also heated until all traces of the 95 acetone have disappeared, after which the phenols are separated from the aqueous layer.

Other solvents which can be mixed with water may however also be used, such as 100 methylated spirit, ethyl alcohol. Of these solvents relatively large quantities are however required in order to dissolve the primary tar free from asphalt. When cooling this solution in addition to the aforementioned slimy substances considerable (methylated anthracene, etc.) quantities of other substances will precipitate so that the yield 105

in pure oil will become considerably less. Apart therefrom the oils obtained in this manner are of a less degree of viscosity, they have however a very good solidifying point 5 ( $-10^{\circ}$  C.) and they are transparent and of a red colour.

Thus by treating the primary tar with acetone the phenols present therein are obtained simultaneously and in great quantities. These phenols owing to their tendency 10 to turn into resins are not suitable to remain in an oil used for lubricating purposes while during the first part of the operation the slimy substances having a great 15 detrimental effect on the solidifying point are divided out.

It has further been proved to be of advantage to free the primary tar prior to removing the asphalt therefrom from water 20 and particularly from the light oil. The latter would make the benzine gradually less suitable to act as a means for removing the asphalt. It has also proved advantageous 25 to drive off the fraction up to  $220$ – $250^{\circ}$  C. in addition to the light oil as the former must in any case be distilled from the lubricating oil in order to increase the viscosity, and to then effect the removal of the asphalt 30 by means of benzine. If the driving off is carried on to a still higher temperature perhaps to a temperature of  $320^{\circ}$  C., where the decomposition of the viscous parts commences, the parts of the tar, which cannot 35 withstand such temperatures polymerize and are also separated out during the subsequent removal of the asphalt. In this manner lubricating oils in lesser yield but of a higher capacity for resisting heat, are obtained.

Instead of the ordinary kinds of benzines 40 (petroleum benzine) other benzines such as primary tar benzines may be used. The latter yield a slightly less quantity of asphalt, the resulting oils are however more viscous, the yield of oil is greater, while the oils obtained therewith can only be used for ordinary and crude lubricating purposes on account of their small contents of soft asphalt.

*Example.*—1100 parts by weight of a primary tar obtained from a gas generator are 50 distilled up to a temperature up to  $240^{\circ}$ , 90 parts by weight of the distillates being obtained. The residue of distillation = 1010 parts by weight is dissolved in double the quantity of benzine by stirring the mixture and the latter is allowed to stand quietly for a period of 24 hours, preferably by cooling it with water or ice, whereupon the benzine solution is poured off from the asphalts and the benzine is distilled off.

60 From 1100 parts of primary tar the following is obtained:

Parts by weight.

1. Distillate up to  $240^{\circ}$  C. = 90
2. Asphalt. = 495
3. Oils free from asphalt. = 515

These 515 parts by weight of oil free from asphalt are dissolved in double the quantity of acetone while the mixture is stirred and cooled by means of ice. 45 parts by weight of a slimy substance are separated and removed from the solution by filtration. By subsequently diluting the acetone solution of the primary tar free from asphalt with approximately 300 parts by weight of water, 70 405 parts of neutral oils free from phenols, 75 separate out. The aqueous acetone solution contains 65 parts by weight of phenols which after driving off of the acetone mostly separate from the watery solution.

The 1100 parts of primary tar thus yield 80

|                                    | Per cent. |
|------------------------------------|-----------|
| 1. Fraction up to $240^{\circ}$ C. | = 8.1     |
| 2. Asphalt.                        | = 45.0    |
| 3. Slimy substances                | = 4.1     |
| 4. Phenols.                        | = 5.9     |
| 5. Lubricating oils                | = 34.5    |
| 6. Losses                          | = 2.4     |

At  $20^{\circ}$  C. the oil has a specific gravity of 1.03, a viscosity =  $8.45^{\circ}$  Engler at  $50^{\circ}$  C., 90 a flash point of  $138^{\circ}$  C. and a solidifying point of  $-4^{\circ}$  C.

The conditions under which the experiments are carried out may according to requirement and to the objects for which the substances are intended, be varied within wide ranges. The result obtained with other primary tars also vary since the quality of the primary tars chiefly depends upon the process of low temperature distillation. 100

The mode of separating the asphaltic material from tar, as herein described, is not claimed herein but forms the subject matter of my concurrent application 755,554.

I claim as my invention:

1. In the process of obtaining lubricating oils and phenols from primary tar, the steps which comprise distilling the tar up to about  $240^{\circ}$  C., adding a quantity of benzine to the still residue in order to separate insoluble asphaltic materials from said residue, separating the insoluble materials from the benzine solution, distilling off the benzine from said solution, adding, to the lubricating oil material remaining, a solvent for said oil material, said solvent being also miscible with water, and thereafter adding water to said so prepared solution whereby the oil is caused to separate out and the phenols remain in solution.

2. In the process of obtaining lubricating oils and phenols from primary tar, the steps which comprise mixing the tar with a quantity of benzine amounting to several times the quantity of the tar, separating the precipitated asphaltic materials from the remaining oil, removing the benzine from the oil by distillation, adding to the oil a solvent for the oil miscible therewith and also miscible with water in sufficient quantity to dis-

solve said oil, adding water to throw the oil out of solution but leaving the phenols in solution, and thereafter separating the oil from the aqueous layer.

5 3. In the process of separating lubricating oils and phenols from oils containing the same and obtained in the treatment of primary tar the steps which comprise adding to the material, which contains the lubricating oils and phenols, a solvent for the material, miscible therewith and miscible with water, adding water to the so prepared solution to throw the lubricating oils out of solution and separating off the aqueous layer 10 containing the phenols.

4. In the process of separating lubricating oils and phenols from oils containing the same and obtained in the treatment of primary tar, the steps which comprise adding acetone to the material, which contains lubricating oils and phenols, in a quantity sufficient to dissolve said material, adding water to the so prepared solution in order to throw out of solution the lubricating oils and separating off the aqueous layer containing the phenols. 20 25

In testimony whereof I affix my signature.

ANTON WEINDEL.